

## UNITED STATES PATENT OFFICE.

CARL PIERCE LEWIS, OF BURLINGAME, CALIFORNIA, ASSIGNOR TO MINERALS SEPARATION NORTH AMERICAN CORPORATION, OF NEW YORK, N. Y., A CORPORATION OF MARYLAND.

## FROTH-FLOTATION CONCENTRATION OF ORES.

No Drawing. Application filed August 4, 1926, Serial No. 127,180, and in Great Britain August 12, 1925.

This invention relates to the froth-flo-  
tation concentration of ores, and is herein illus-  
trated as applied to the differential flotation  
of lead-zinc ores, for the collection of a lead  
5 concentrate with the separate collection of  
a zinc concentrate, if desired.

According to the present invention a froth  
concentrate is separated by the aid of a flo-  
tation agent which is mainly composed of a  
10 soluble mineral-frothing agent, such as cre-  
syllic acid or steam distilled pine oil, thereby  
floating the desired value, nearly free from  
any other normally floatable material. A  
15 modifying agent, such as a cyanide, may be  
used in addition to this flotation agent to in-  
hibit the flotation of the other material, thus  
for example facilitating the separation of  
lead from zinc. The flotation agent used for  
20 producing a second froth may also be mainly  
composed of a soluble mineral-frothing agent,  
such as cresyllic acid, or steam distilled pine  
oil; and other agents may be used therewith.  
In this way a large recovery of an exceed-  
25 ingly rich lead concentrate may often be ef-  
fected. Any iron present may be largely  
kept out of both the concentrates.

*Example 1.*—Low grade ore from Keno  
Hill, Alaska, was made into a pulp with water  
and agitated with 0.15 pounds potassium cy-  
30 anide, 0.10 pounds potassium xanthate, and  
0.20 pounds cresyllic acid, all per ton of ore,  
and a lead-bearing froth separated. The re-  
sults are shown in the following table, from  
35 which it will be seen that a large recovery of  
the lead was effected in an exceedingly rich  
concentrate, and that there was substantially  
no concentration of the zinc with the lead.

|               | Assays |       |       | Recoveries |       |
|---------------|--------|-------|-------|------------|-------|
|               | Wt. %  | Pb. % | Zn. % | Pb. %      | Zn. % |
| Heads.....    | 100.   | 4.86  | 3.5   | 100.       | 100.  |
| Pb. conc..... | 6.4    | 73.0  | 3.6   | 96.2       | 6.6   |
| Pb. tail..... | 93.6   | .2    | 3.5   | 3.8        | 93.4  |

*Example 2.*—A pulp of an iron-bearing  
lead-zinc ore from Mexico was agitated with  
0.7 pounds of potassium xanthate, and 0.10  
pounds cresyllic acid, both per ton of ore to  
50 yield a lead concentrate, and then further  
agitated with 4 pounds of lime, 1.2 pounds  
copper sulphate, 0.2 pounds of potassium  
xanthate, and 0.15 pounds of steam distilled  
pine oil, all per ton of ore, and a zinc concen-

trate separated. The results are shown in 55  
the following table.

|               | Assays |       |       | 60 |
|---------------|--------|-------|-------|----|
|               | Pb. %  | Zn. % | Fe. % |    |
| Heads.....    | 11.3   | 23.9  | 4.7   |    |
| Pb. conc..... | 68.0   | 14.0  |       |    |
| Zn. conc..... | 3.4    | 60.0  |       |    |
| Tails.....    | .6     | 1.7   |       |    |

*Example 3.*—A pulp of Nevada lead-zinc  
ore, carrying some silver was similarly agi-  
tated with the same agents in the same pro-  
portion, to yield a lead concentrate and a  
zinc concentrate, the results being shown in  
70 the following table:

|               | Assays  |       |       | 75 |
|---------------|---------|-------|-------|----|
|               | Ag. oz. | Pb. % | Zn. % |    |
| Heads.....    |         |       |       |    |
| Pb. conc..... | 25.9    | 10.8  | 11.9  |    |
| Zn. conc..... | 6.7     | 1.2   | 50.2  |    |
| Tails.....    | .10     | 0.4   | 1.2   |    |

The indicated recovery of the lead in the 80  
lead concentrate was 95.5%.

*Example 4.*—A pulp of ore from Federal  
Morning Mine ore was agitated with po-  
tassium cyanide 0.15 pounds, potassium xan-  
thate 0.05 pounds, and cresyllic acid 0.1 pound,  
85 all per ton of ore, and a lead-bearing froth  
was separated. The pulp was then further  
agitated with the further addition of copper  
sulphate 0.6 pounds, lime 6 pounds, potassium  
xanthate 0.2 pounds, and steam distilled pine 90  
oil 0.15 pounds, all per ton of ore, and a  
zinc-bearing froth separated partly as a fin-  
ished concentrate and partly as a middling.  
The results are shown in the following table:

|               | Assays |       |       | 95 |
|---------------|--------|-------|-------|----|
|               | Pb. %  | Zn. % | Fe. % |    |
| Heads.....    | 17.5   | 9.0   | 21.   |    |
| Pb. conc..... | 64.4   | 9.6   | 6.    |    |
| Zn. conc..... | 9.5    | 50.0  | 8.    |    |
| Zn. Midd..... | 18.6   | 4.6   | 25.6  |    |
| Tails.....    | 2.4    | .4    | 30.4  |    |

Having thus described certain embodi-  
ments of my invention what is claimed is:

1. The process of concentrating an ore con-  
taining a floatable value and another nor-  
mally floatable material which consists in

- agitating a pulp of the ore with a xanthate and with a flotation agent mainly composed of soluble mineral-frothing agent, to yield a froth rich in the floatable value, separating
- 5 the froth, further agitating with the addition of a further agent adapted to facilitate the floating of the other normally floatable material so as to yield a froth rich in said other normally floatable material, and separating
- 10 the froth.
2. A process of concentrating a lead-zinc ore which consists in agitating a pulp of the ore with a xanthate and with a flotation agent mainly composed of soluble-mineral froth-
- 15 ing agent, to yield a froth rich in lead, sepa-
- rating the froth, further agitating with the addition of a further agent adapted to facilitate the floating of the zinc so as to yield a froth rich in zinc, and separating the froth.
3. A process of concentrating a lead-zinc ore which consists in agitating a pulp of the ore with a xanthate and cresylic acid to yield a froth rich in lead, separating the froth, further agitating with the addition of pine oil to yield a froth rich in zinc, and sep- 25 arating the froth.
- In testimony whereof, I have affixed my signature to this specification.

CARL PIERCE LEWIS.